

## UNITED STATES PATENT OFFICE

2,637,634

## ALUMINUM ETCH

Roscoe D. Howard and Robert E. Samuelson,  
Wichita, Kans., assignors to Beech Aircraft  
Corporation, Wichita, Kans., a corporation of  
Delaware

No Drawing. Application February 12, 1952,  
Serial No. 271,292

1 Claim. (Cl. 41—42)

1

The invention disclosed in this patent relates to the etching and cleaning of aluminum alloys preparatory to shielded arc welding or to electrical resistance welding, such as spotwelding and seam welding.

Objects of the invention are to effect rapid, uniform chemical cleaning in a single dip operation, at room temperature and under generally practical and economical operating conditions.

Special objects of the invention are to insure accomplishment of better, stronger welds, faster welding operations, a greater number of welds between tip cleanings, consistency of welds at prescribed machine settings, top quality welds of shielded arc weld machines, less "down" time for cleaning electrode tips and machine adjustments, and generally improved welding conditions.

The invention is particularly directed toward the treatment of more refractory aluminum alloys associated with aircraft, especially that identified as 61S. The heat treating operation on this particular aluminum alloy has the effect of creating a dense refractory coating, difficult of removal by known etching operations.

It has been a purpose of the present invention to provide an etch which would remove such dense refractory coatings without injuring the metal surface and which would leave the surface chemically clean, smooth and hard, ready for uniform spotwelding and inert gas shielded arc welding operations.

Other desirable objects attained by the invention and the novel features constituting the invention are set forth and will appear in the course of the following specification.

In developing an etch which would accomplish the foregoing, it was determined that the fluoride ion, in some combination, was essential to satisfactory results.

Commercial grades of hydrofluoric acid (48-52%) may be used. Dilute solutions of hydrofluoric acid vigorously attack aluminum alloys but in addition cause deposition of a thin, loosely adherent layer of a black to brownish-black smut.

Addition of nitric acid, up to about 20% or more by volume, to an approximate 3% by volume, hydrofluoric acid solution constrains or restrains the vigorous action of the fluoride ion and to an extent retards the smut formation.

2

Addition of boric acid to the nitric hydrofluoric combination effects a still further leveling action and eliminates the smut formation.

The amount of boric acid, either powder or crystals, may be approximately 1% by weight.

This combined nitric-hydrofluoric-boric acid combination in the approximate ratios stated, is especially effective in removing the dark, dense, refractory coating resulting from the heat treating operation on 61S aluminum alloy.

A single dip with an immersion time of four minutes has been found ample even for the most refractory parts.

This operation may be carried on at normal room temperatures and even ranging as high as 130° F.

The cost per unit treated is low and the solution may be rejuvenated and balanced as it is expended through usage.

20 The corrosive character of the solution requires care in handling. Tank linings of "Koroseal" and carbon brick may be used and effective surface exhaustion of vapors and gases evolved, may be employed.

25 Examples of properly balanced and buffered solutions necessary for smooth, bright, hard, smut-free surfaces of aluminum alloy products, are given as follows:

30 1. By percentage figures—

Nitric acid, sp. gr. 1.42, 20% by volume  
Hydrofluoric acid (50% conc.), 3% by volume  
Boric acid (powdered or crystal), 1% by weight  
Water to make 100% by volume

35 2. By volume and weight figures—

To make 3,000 gallons:

35 Nitric acid, 42° Bé. (67-68% HNO<sub>3</sub>), 600 gallons  
Hydrofluoric acid (50%), 90 gallons (see Note 1)  
Boric acid, 280 pounds (see Note 2)  
Water to make 3,000 gallons solution

40 NOTE 1.—When 60% hydrofluoric acid is used instead of the 50% type, a total of only 75 gallons will be required to supply the correct fluoride concentration.

NOTE 2.—Secure complete solution of the boric acid before etching any parts in the tank.

45 Cooling water may be run through a jacketed section of the tank to keep the solution operating at room temperatures, say up to 130° F., and the action may be governed to avoid going above such temperature.

50 The invention is particularly suited to conveyorized operations, with the material or objects transported by conveyor through the tank

at a rate for approximately four minutes immersion.

Various concentrations of acid may be used, but the approximate ratio of nitric acid to hydrofluoric acid to boric acid given should be maintained.

Rejuvenation may be effected at regular periods as by addition, say, of one-third each of the original chemicals, such as:

Nitric acid -----  $\frac{1}{3} \times 600 = 200$  gallons  
 Hydrofluoric acid -----  $\frac{1}{3} \times 90 = 30$  gallons  
 or, (if 60% sol. used) -----  $\frac{1}{3} \times 75 = 25$  gallons  
 Boric acid -----  $\frac{1}{3} \times 280 = 93$  pounds

A measure of the quality of the chemical cleaning effected may be determined by the surface resistance as expressed in microhms.

The etch described gives surface readings of 10 or less microhms, and this will give 150 or more spots, meeting all specification requirements, between tip cleanings, and much higher production than possible with currently available etches.

Consistency attained in the pretreatment described results in consistency of welds at prescribed machine settings. The solution made up in the ratios disclosed is so balanced as to yield surfaces having consistent microhm resistance readings, enabling greatly increased number of spotwelds between tip cleanings.

Greater economy of operation also results from the fact that it may not be necessary, for chemical reasons, to discard an entire batch of etch solution, because the drag-in and drag-out plus the additions of make-up permits practically continuous operation with the solution until such time as possibly mechanical failure or maintenance reason may necessitate shut-down and complete dumping of a batch.

10 While particularly useful for 61S aluminum alloy, the invention, it will be realized, is adapted to the treatment of various other aluminum alloys.

What is claimed is:

15 Aluminum etch comprising the following in approximately the proportions:

Nitric acid, 42° Bé ----- 20 gallons  
 Hydrofluoric acid (48-52% HF) ----- 3 gallons  
 Boric acid ----- 9.3 pounds  
 Water to make 100 gallons total.

ROSCOE D. HOWARD.  
 ROBERT E. SAMUELSON.

References Cited in the file of this patent

UNITED STATES PATENTS

| Number       | Name      | Date          |
|--------------|-----------|---------------|
| 2,409,271    | Goldowski | Oct. 15, 1946 |
| 2,465,750    | Reid      | Mar. 29, 1949 |
| 30 2,593,447 | Hesch     | Apr. 22, 1952 |